

July 11, 1939.

L. C. JONES ET AL

2,165,797

PHOTOGRAPHIC DEVELOPERS

Filed July 13, 1938

4 Sheets-Sheet 1



FIG. 2.



FIG. 1.

INVENTORS.  
LOUIS C. JONES  
ROBERT DANLING BARNES  
GARNET PHILIP HAN

*Robert Danling Barnes*  
ATTORNEY.

July 11, 1939.

L. C. JONES ET AL

2,165,797

PHOTOGRAPHIC DEVELOPERS

Filed July 13, 1938

4 Sheets-Sheet 2



FIG. 4.



FIG. 3.

INVENTORS.

LOUIS C. JONES  
ROBERT BOYLING BARNES  
GARNET PHILIP HAM

BY

Robert L. Mather  
ATTORNEY.

July 11, 1939.

L. C. JONES ET AL  
PHOTOGRAPHIC DEVELOPERS

2,165,797

Filed July 13, 1938

4 Sheets-Sheet 3



FIG. 6.



FIG. 5.

INVENTORS.  
LOUIS C. JONES  
ROBERT BOWLING BARNES  
GARNET PHILIP HAM

*Robert Ames Norlin*  
ATTORNEY.

July 11, 1939.

L. C. JONES ET AL

2,165,797

PHOTOGRAPHIC DEVELOPERS

Filed July 13, 1938

4 Sheets-Sheet 4



FIG. 7.

INVENTORS.

LOUIS C. JONES  
ROBERT BOYLING BARNES  
GARNET PHILIP HAM

BY

*Robert Ames Morton*  
ATTORNEY.

Patented July 11, 1939

2,165,797

# UNITED STATES PATENT OFFICE

2,165,797

## PHOTOGRAPHIC DEVELOPER

Louis C. Jones, Greenwich, Robert Bowling Barnes, Stamford, and Garnet Philip Ham, Old Greenwich, Conn., assignors to American Cyanamid Company, New York, N. Y., a corporation of Maine

Application July 13, 1938, Serial No. 218,972

4 Claims. (Cl. 95—88)

This invention relates to photographic developers, and more particularly to developers for photographic negatives which are capable of variation of contrast.

5 The ordinary type of photographic developer of which the Metol-hydroquinone types are the most common normally contain at least three types of ingredients; the actual developers such as Metol, hydroquinone and the like, protective 10 agents against oxidation such as sodium sulfite, and a suitable alkali to produce a pH suited for the particular developer. In addition, other ingredients such as restrainers, for example alkali metal bromides and in the case of tropical 15 developers, sodium sulfate, may be present. Normally, a developer formula is balanced with regard to the three main ingredients in order to give good results and produce a satisfactory fidelity in reproducing the various gradations of 20 light and shadow of the object photographed. When a curve is constructed having ordinates proportional to the density of the final developed negative, that is to say, the negative logarithm of the transmission and with abscissae proportional 25 to the logarithm of exposure, there should be a long, reasonably straight portion of the curve in order to reproduce with reasonable fidelity various exposures within a certain range. With most modern developers, satisfactory fidelity is ob- 30 tained, but a relatively large number of formulae are in use because it is difficult to change the characteristics of a particular formula without upsetting its balance.

A few years ago, a new alkali consisting of a 35 mixture of alkaline substances, notably borates, was introduced by the Eastman Kodak Company under the name "Kodalk", and is covered by U. S. Patent No. 1,990,800. Four different formulae of the Eastman Kodak Company, namely 40 DK-15, DK-50, DK-60 and DK-76, have been formulated using the new alkali and claims have been made for "Kodalk" that contrast can be varied within wide limits by variation in the amount of alkali without upsetting the balance 45 of the developer, thus producing results which give poor fidelity. This is an important advantage as it makes possible the use of a relatively small number of formulae for a wide number of purposes since it is possible to vary the contrast 50 within considerable limits by variation of the alkali component without requiring a complete recalculation of the entire formula.

While "Kodalk" possesses the properties claimed for it to a considerable degree and thus 55 represents a distinct advance over the use of standard alkalies such as sodium carbonate, in some formulae it leaves much to be desired. Its change in contrast is sometimes accompanied by a loss of fidelity. According to the present in- 60 vention, it has been found that a new class of

bases which can be used to supply the alkaline reaction necessary for most photographic developers possesses the advantages of variation in contrast with variation in amount of the base, and in some formulae the best of them are superior in this respect to "Kodalk". The compounds of the present invention are those of the very strong organic bases, namely, the quaternary ammonium compounds and the amidines. The quaternary ammonium compounds may be 10 used in the form of their free bases, but the amidines are normally used in the form of their salts with weak acids such as carbonic acid. Among the most effective of the compounds of the present invention are guanidine carbonate 15 and trimethylbenzylammonium hydroxide, known to the trade as "Tetrone B", the former giving the best results of any of the organic bases tested.

The invention will be described in detail in 20 conjunction with specific examples illustrating the use of the compounds of the present invention in typical Metol-hydroquinone developer formulae. The compounds are also useful in other types of developers such as those using 25 p-phenylene diamine and glycine, but are of less importance with this class of developers which are normally used at low contrast to produce extreme fine grain. The invention will also be described in conjunction with curves showing the 30 results of densitometric measurements on exposed negatives which are illustrated on the drawings in which

Fig. 1 represents curves with a DK-15 type developer; 35

Fig. 2 is a series of curves with a DK-50 type developer;

Fig. 3 is a series of curves with a DK-60 type developer;

Fig. 4 is a series of curves with a DK-76 type developer; 40

Fig. 5 is a series of curves with various developers using sodium carbonate as an alkali;

Fig. 6 is a series of curves with various developers using a 50%-50% mixture of sodium carbonate and guanidine carbonate as alkalies; and 45

Fig. 7 is a series of curves comparing "Tetrone B" and guanidine borate.

### EXAMPLE 1

An ordinary DK-15 developer was made up as follows:

|                      |                   |       |    |
|----------------------|-------------------|-------|----|
| Water                | cubic centimeters | 500   | 55 |
| Metol                | grams             | 2.85  |    |
| Sodium sulfite, des. | do                | 45.00 |    |
| "Kodalk"             | do                | 11.25 |    |
| Potassium bromide    | do                | 0.95  |    |
| Sodium sulfate       | do                | 22.50 | 60 |

and a second batch was made up with guanidine carbonate as follows:

|                      |                   |       |
|----------------------|-------------------|-------|
| Water                | cubic centimeters | 500   |
| Metol                | grams             | 2.85  |
| Sodium sulfite, des. | do                | 45.00 |
| Guanidine carbonate  | do                | 8.80  |
| Potassium bromide    | do                | 0.95  |
| Sodium sulfate       | do                | 22.50 |

10 This type of developer is intended for tropical development of general film, and has a pH of approximately 9.2. The amount of guanidine carbonate used was sufficient to give a similar pH.

A third batch of developer was made up with 15 five times the amount of "Kodalk" and its pH measured 10.17. Thereupon a fourth developer was made up with an amount of guanidine carbonate sufficient to give a similar pH. This contained slightly less than five times the weight 20 of guanidine carbonate in the second developer.

A photographic wedge made by the Eastman Kodak Company and having nine steps between light and dark arranged logarithmically, each 25 step from dark to light representing a transmission 150% that of the preceding step, was used to make exposures on 35 mm. Eastman Kodak supersensitive panchromatic film. This film was chosen as being representative of a medium fast, long latitude panchromatic film which would 30 show up lack of fidelity or excessive fogging rapidly and which is a type of film where variations in contrast produced by the developer are normally most necessary. All exposures were carefully calibrated using a Leitz enlarger with 35 a 10 watt bulb and lens stopped down to F12.5 as a source of illumination. All conditions of development including time, temperature, agitation, fixing, washing and the like were kept uniform and the only difference between the tests 40 was the developer type used. Densitometric measurements were made in a photoelectric densitometer calibrated against the wedge used for the exposures. The results appear on the curves in Fig. 1 of the drawings. It will be noted 45 that in this ultra high speed tropical developer, both "Kodalk" and guanidine carbonate gave excellent results, both in normal amounts and when five times normal amounts were used. A sharp 50 increase in the contrast as shown by the greater steepness of the curve was observed but the straight portions of both sets of curves assure satisfactory fidelity.

A test was then made of the keeping qualities 55 of the developers having five times the amount of base and here a very sharp difference was noted. The guanidine carbonate after 20 days showed results substantially similar to a fresh normal guanidine carbonate developer, whereas 60 the "Kodalk" had lost its fidelity and gave a curve of irregular shape.

#### EXAMPLE 2

65 Four developers were prepared according to Eastman Kodak formula DK-50 as follows, the first having the normal amount of "Kodalk" and giving a pH of 9.12, the second having the required amount of guanidine carbonate to give the 70 same pH and two others, one of which contained five times the amount of "Kodalk" and the other an amount of guanidine carbonate less than five times as much, but which gave a slightly higher pH. The actual amount was only 3 1/2 75 times as much as that used in the normal solution.

#### Formula 1

|                      |                   |       |
|----------------------|-------------------|-------|
| Water                | cubic centimeters | 500   |
| Metol                | grams             | 1.25  |
| Sodium sulfite, des. | do                | 15.00 |
| Hydroquinone         | do                | 1.25  |
| "Kodalk"             | do                | 5.00  |
| Potassium bromide    | do                | 0.25  |

#### Formula 2

|                      |                   |       |
|----------------------|-------------------|-------|
| Water                | cubic centimeters | 500   |
| Metol                | grams             | 1.25  |
| Sodium sulfite, des. | do                | 15.00 |
| Hydroquinone         | do                | 1.25  |
| Guanidine carbonate  | do                | 3.30  |
| Potassium bromide    | do                | 0.25  |

This formula is one used for the development of normal films of both orthochromatic and panchromatic type. The results obtained are shown in the curves of Fig. 2 from which it is apparent 20 that the contrast with guanidine carbonate is slightly greater than with "Kodalk" and that when five times the amount is used, a much better curve of higher contrast was obtained with 25 guanidine carbonate.

Again a keeping test was carried out, and the results were similar to those observed with DK-15; that is to say, the guanidine carbonate returned to the characteristics of the normal developer, whereas the "Kodalk" lost its fidelity. 30

#### EXAMPLE 3

Four developers were prepared according to Eastman Kodak formula DK-60 as follows, the first having the normal amount of "Kodalk" and 35 giving a pH of 9.43, the second having the required amount of guanidine carbonate to give the same pH, and two others, one of which contained five times the amount of "Kodalk" and the other an amount of guanidine carbonate 40 which gave a slightly higher pH. The actual amount used was only 4 1/2 times as much as that used in the normal solution.

#### Formula 1

|                      |                   |       |
|----------------------|-------------------|-------|
| Water                | cubic centimeters | 500   |
| Metol                | grams             | 1.25  |
| Sodium sulfite, des. | do                | 15.00 |
| Hydroquinone         | do                | 1.25  |
| "Kodalk"             | do                | 10.00 |
| Potassium bromide    | do                | 0.25  |

#### Formula 2

|                      |                   |       |
|----------------------|-------------------|-------|
| Water                | cubic centimeters | 500   |
| Metol                | grams             | 1.25  |
| Sodium sulfite, des. | do                | 15.00 |
| Hydroquinone         | do                | 1.25  |
| Guanidine carbonate  | do                | 6.80  |
| Potassium bromide    | do                | 0.25  |

This developer is also intended for general development of films of both the orthochromatic and panchromatic type where a somewhat higher contrast is desired. The results are shown in Fig. 3. Again it will be noted that the increase in contrast is substantially the same with guanidine carbonate and with "Kodalk" but on keeping, the "Kodalk" loses fidelity whereas the guanidine carbonate assumes a position intermediate between that of the fresh normal developer and 70 that of the fresh developer with five times the base. The curve, however, shows a long straight portion retaining the excellent fidelity characteristics which are typical of the guanidine carbonate developers.

## EXAMPLE 4

Four developers were prepared according to Eastman Kodak formula DK-76 as follows, the first having the normal amount of "Kodalk" and giving a pH of 8.51, the second having the required amount of guanidine carbonate to give the same pH and two others, one of which contained five times the amount of "Kodalk" and the other amount of guanidine carbonate which gave a slightly higher pH. The actual amount used was slightly more than five times as much as that used in the normal solution. This was necessary because of the shape of the pH curve of guanidine carbonate at lower concentrations.

15

## Formula 1

|                      |                   |      |
|----------------------|-------------------|------|
| Water                | cubic centimeters | 500  |
| Metol                | grams             | 1.0  |
| Sodium sulfite, des. | do                | 50.0 |
| Hydroquinone         | do                | 2.5  |
| "Kodalk"             | do                | 1.0  |

## Formula 2

|                      |                   |      |
|----------------------|-------------------|------|
| Water                | cubic centimeters | 500  |
| Metol                | grams             | 1.0  |
| Sodium sulfite, des. | do                | 50.0 |
| Hydroquinone         | do                | 2.5  |
| Guanidine carbonate  | do                | 1.3  |

30 The results are shown on the curves of Fig. 4. The guanidine carbonate gave somewhat greater contrast than "Kodalk", but in this developer the keeping qualities of the "Kodalk" are improved.

## EXAMPLE 5

35 In order to obtain a comparison with an alkali which does not permit wide variations, sodium carbonate was substituted for the "Kodalk" and guanidine carbonate in five times normal strength and results are shown in Fig. 5. It will be noted that only in DK-15 is there any approach to a curve of satisfactory fidelity.

## EXAMPLE 6

40 A surprising result is obtained when mixtures of guanidine carbonate and sodium carbonate are used. The mixtures appear to have substantially the desirable characteristics of guanidine carbonate alone. The formula DK-50 type was prepared substituting the mixture for the five times value in Example 2, and the results for various mixtures are shown in the curves in Fig. 6 which

should be compared with the curve for sodium carbonate alone with DK-50 in Fig. 5. It will be noted that while all of the curves show satisfactory fidelity, the good contrast with best fidelity is obtained with the 50%-50% mixture of guanidine carbonate and sodium carbonate. The particular proportions are, however, not critical which is an advantage. The possibility of substituting sodium carbonate for a considerable part of the guanidine carbonate represents a real 10 commercial advantage because of the lower price of the sodium carbonate as contrasted with guanidine carbonate or with "Kodalk".

## EXAMPLE 7

15 DK-50 and DK-76 formulae were prepared with five times normal "Kodalk" and with five times normal trimethylbenzylammonium hydroxide ("Tetron B"). DK-50 was also prepared with five times normal guanidine borate. 20 The results appear in Fig. 7. It will be noted that "Tetron B" gave results similar to "Kodalk" in the case of DK-50 with slightly less contrast but somewhat better fidelity. The results of the DK-76 show excellent fidelity but less contrast. 25 Guanidine borate, due to its relative insolubility, could not be used to produce the desired pH. The developer solution produced a pH of only 8.8 in place of a normal 9.98. It will be noted that the curve does not show as high contrast which, of course, is to be expected as the necessary alkalinity could not be reached with this compound.

30 What we claim is:

1. A photographic developer for silver halides containing as its alkalinity producing agent 35 guanidine carbonate.
2. A metol-hydroquinone photographic developer containing as its alkalinity producing agent guanidine carbonate.
3. A photographic developer containing as its 40 alkalinity producing agent a mixture of sodium carbonate and guanidine carbonate in effective amounts.
4. A metal-hydroquinone photographic developer containing as its alkalinity producing 45 agent a mixture of sodium carbonate and guanidine carbonate in effective amounts.

LOUIS C. JONES,  
ROBERT BOWLING BARNES. 50  
GARNET PHILIP HAM.